

Jan. 16, 1962

M. J. SAARIVIRTA

3,017,268

COPPER BASE ALLOYS

Filed May 9, 1960



INVENTOR  
MATTI J. SAARIVIRTA

BY  
Kasper T. Serjan  
ATTORNEY

## 1

3,017,268

### COPPER BASE ALLOYS

Matti J. Saarivirta, Plainfield, N.J., assignor to American Metal Climax, Inc., New York, N.Y., a corporation of New York

Filed May 9, 1960, Ser. No. 27,680  
8 Claims. (Cl. 75—154)

This invention relates to copper base alloys essentially containing titanium, tin and chromium. The alloys of this invention have a minimum copper content of 90% and are age hardenable. They possess highly desirable properties attained preferably by working and heat treatment which properties make the material particularly suitable for various electrical and electronic applications including the making of electrodes and their holders for resistance welding machines, electrical contacts, springs and numerous other items requiring reasonably good strength, conductivity, ductility, resistance to corrosion and stability to the extent that the desirable properties and characteristics of the alloy are retained at elevated temperatures.

For the making of springs, contactors and the like, age hardenable copper base alloys containing beryllium are used quite extensively. Commercially available beryllium alloys containing, for example, 0.4 to 0.7% beryllium, 2.3 to 2.7% cobalt, balance copper possess attractive mechanical properties in several respects including a tensile strength of as much as 100,000 p.s.i. combined with electrical conductivity of about 48% that of pure copper. Such a combination of properties are exceedingly difficult to obtain since in the case of most copper alloys having a tensile strength of about 90,000 to 100,000 p.s.i. or higher, the electrical conductivity is rarely above 30% that of pure copper.

Although the aforesaid beryllium-copper alloys are satisfactory for various electrical and electronic applications with respect to meeting mechanical and physical property requirements not met by most other copper base alloys, such alloys have the drawback that they are rather difficult and costly to make. Furthermore, these alloys require the use of beryllium which in addition to being expensive is also an extremely toxic substance necessitating special precautions in the making and subsequent processing of such alloys. Then too, whereas such beryllium copper alloys are suitable for rather limited high temperature applications, extreme brittleness is encountered at temperatures in excess of about 225—250° C. leading to failure of the alloy. Accordingly, there is an urgent need for materials which not only possess satisfactory properties at ordinary temperatures of operation but which also are capable of withstanding higher temperatures over prolonged periods of operation without excessive deterioration of the alloy by embrittlement or otherwise.

It has now been discovered that quaternary alloys of copper containing titanium, tin and chromium which alloying ingredients are present in relatively small amounts not exceeding 10% in the aggregate provide age hardenable copper base alloys that can be readily processed by appropriate treatment to provide physical and mechanical properties that compare favorably by comparison with the aforesaid beryllium-containing copper base alloys. The new and novel alloys of this invention not only possess satisfactory properties and characteristics at ordinary

## 2

temperatures of operation but are also markedly superior with respect to their ability to withstand significantly higher temperatures without failure. The alloys of the present invention have the further important advantage of being much more economical to produce than the previously mentioned copper-beryllium-cobalt alloys. At the same time, the serious toxicity problems associated with the use of beryllium are completely eliminated.

It is therefore, an object of this invention to provide copper-titanium-tin-chromium alloys possessing excellent mechanical properties and characteristics for applications and uses requiring a copper base alloy of medium strength and reasonably good electrical conductivity.

It is another object of this invention to provide age hardenable copper-titanium-tin-chromium alloys that possess improved properties compared with beryllium-copper alloys especially with respect to retention of said properties under service conditions involving elevated temperatures appreciably higher than 250° C.

Another object of this invention is to provide new and novel alloys that substantially meet the requirements with respect to tensile strength, electrical conductivity and other properties satisfied by beryllium-coppers without incurring the high cost of production and toxicity problems associated with such beryllium-containing alloys.

Other objects and advantages will become readily apparent as this specification proceeds.

The copper base quaternary alloys of this invention generally contain from 0.3 to 4% titanium, 0.5 to 5% tin, 0.05 to 2% chromium, the balance being copper which is present in all instances in the amount of at least 90% with respect to the overall alloy composition. Phosphorus and/or silver may be optionally included in amounts not exceeding 0.05 and 1% respectively without significantly altering the properties of the resulting alloys although the presence of phosphorus in amounts appreciably above 0.02% does effect some reduction in the electrical conductivity of the material. The preferred composition of the quaternary alloy consists of from 1 to 3% titanium, 2 to 4% tin and 0.2 to 0.8% chromium, balance copper, with the proportion of titanium to tin being in the ratio of approximately 1:1.7 respectively. Optimum properties of the alloy are obtained with the use of from 1.3 to 1.7% titanium, 2.2 to 2.9% tin and 0.3 to 0.6% chromium. All of the foregoing percentages refer to the actual content of the various alloying elements in the resulting alloy product.

Although tough pitch copper may be used in making the alloys of the present invention, it is definitely preferred to make said alloys with initially oxygen-free copper. Such coppers include electrolytic cathode copper, copper made in a reducing atmosphere such as OFHC brand copper, or copper made using an inert atmosphere, a vacuum or under a charcoal cover. Chemically de-oxidized copper obtained by the treatment of oxygen-containing copper with phosphorus, lithium or other de-oxidizers may also be used in making said alloys.

The alloys can be made according to standard alloying methods such as melting the copper in an induction furnace and adding the desired amounts of titanium, tin and chromium and possibly other ingredients such as silver and phosphorus when the melt is at a temperature of about 1300° C. The alloying ingredients may be in any form suitable for alloying purposes such as metal sponge, master alloys, etc. If desired, the chromium may be included

in appropriate amount in the form of a copper master alloy (5% Cr) along with the copper at the time of preparing the copper melt in which event only the titanium and tin need be subsequently added. If desired, phosphorus-deoxidized or phosphorized copper may be used in preparing the initial melt whereby the separate addition of phosphorus at a later time need not be made if phosphorus is to be included in the alloy. After alloying, the temperature of the melt is lowered and held at about 1200° C. with the alloy being stirred and allowed to settle for about 5-10 minutes after which it is cast in accordance with conventional practices.

In making the alloy, it is important that an inert protective atmosphere consisting of argon, helium or other inert gas be used throughout the entire operation including the casting step. The use of non-oxidizing gases such as carbon monoxide, nitrogen or hydrogen should be avoided since such gases react in varying degrees with one or more of the alloying ingredients and especially with titanium. If carried out correctly, the melting, alloying and casting procedure presents no difficulties and sound castings are readily produced using copper or any other suitable molds in casting the alloy.

Microscopic study of the cast structure of representative quaternary alloys containing, for example, 1.5% titanium, 2.5% tin and varying amounts of chromium ranging from 0.06 to 1.6% revealed the presence of three phases consisting of the alpha phase, a second phase consisting of Ti-Sn rich compound and a third phase which closely resembles in color and appearance the chromium-rich phase found in the copper-chromium binary alloys. It was observed that the amount of the third phase was increased upon increasing the chromium content of the quaternary alloy. These observations indicated that chromium does not combine with titanium and tin present in the system but forms a compound with copper and, for best results, the chromium content of the alloy should be a minimum of 0.3%. It was also ascertained that this third phase becomes substantially completely dissolved by solution annealing the alloy at about 875° C.

The alloys of the present invention possess excellent hot workability upon being preheated at about 800 to 850° C. said hot working being effected either by hot rolling or forging as may be desired. By way of illustration, a 300 pound casting in the form of an 8 inch diameter billet was readily hot forged after preheating for one hour into square rod material of 2.5 and 1.5 inch sizes respectively with no difficulty. The alloys may also be readily cold worked to reductions up to 90% and even higher by rolling or wire drawing without difficulty.

The conventional heat treatments used to obtain age hardening in copper alloys may be satisfactorily used to harden the alloys of the present invention. Solution annealing is effected by heating the alloy to temperatures generally ranging from about 825 to 890° C. for from a few minutes to about an hour or so depending on the solution annealing temperature used, it being preferred, however, to utilize a temperature between 850 and 885° C. and optimally about 875° C. for about 30 minutes after which the alloy is quenched. Age hardening for from 2 to 4 hours at temperatures generally between 400 and 475° C. and preferably at about 450° C. is conducive to development of maximum strength. If electrical conductivity of about 40 to 50% I.A.C.S. is required as an essential property of the alloy, the optimum combination of properties with respect to strength and conductivity are produced by extending the heat treatment period to generally from 6 to 8 hours utilizing the preferred age hardening temperature of about 450° C. Cold working by wire drawing prior to precipitation hardening of the alloy appreciably reduces the aging time required for development of optimum properties including electrical conductivities between 40 and 50%.

The cast alloy processed, for example, by solution annealing at 875° C. for from 15 to 30 minutes, quenched in

water and age hardened for from 6 to 14 hours at 450° C. possesses a tensile strength ranging from 60,000 to 80,000 p.s.i., electrical conductivity of from 35 to 50% I.A.C.S. and elongation values (percent in 2 inches) up to 10%. Prior to age hardening, the tensile strength of the solution annealed material generally ranges from 45,000 to 55,000 p.s.i., the electrical conductivity is only about 7% I.A.C.S. and elongation is about 40% with reference to a representative alloy of the same composition containing 1.5% titanium, 2.5% tin, 0.5% chromium, balance copper.

The alloys of the present invention are readily processed from cast material into wrought products such as bar stock, wire, sheet material, etc. utilizing typical processing steps consisting of (a) preheating the cast alloy at 800 to 850° C., (b) hot working as by rolling or forging, (c) solution annealing at about 875° C. for about 30 minutes, (d) quenching, and (e) age hardening at about 450° C. for about 6 to 8 hours. Cold working with intermediate annealing may be additionally included in the processing steps with the alloy being subjected to precipitation hardening either in the cold worked state or in the solution annealed condition following quenching.

In the accompanying drawing, the effect of age hardening solution annealed wire of nominal composition (1.5% Ti, 2.75% Sn, 0.6% Cr, balance Cu) for varying periods of time at 450° C. is graphically shown with reference to various properties of the alloy. In these tests a 1 inch diameter casting was preheated at 850° C., hot rolled to 0.25 inch diameter rod, annealed at 875° C. for 30 minutes, quenched, cold drawn to 0.132 inch diameter wire and solution annealed at 875° C. for 30 minutes. Specimens of the solution annealed material were then subjected to aging at 450° C. for varying periods of time up to a maximum of 14 hours as indicated in the drawing. The FIGURE shows that maximum precipitation hardening of the alloy occurs during the second through fourth hours of heat treatment but the electrical conductivity is only 20 to 25% I.A.C.S. with such heat treatment. Overaging occurs after 4 hours with some loss of tensile strength but with an increase in elongation and conductivity values with the optimum combination of properties being obtained after aging for 6 to 8 hours. In this condition tensile and yield strengths of about 95,000 and 70,000 p.s.i. respectively, elongation of from 13 to 16% and electrical conductivity values of from 40 to 46% I.A.C.S. are characteristic properties of the alloy. Hardness values of this representative alloy range from 75 VPN in the solution annealed condition to about 200 VPN after aging for 8 hours.

Tensile strengths appreciably above 100,000 p.s.i. with electrical conductivity better than 40% are readily obtained by aging the alloy after cold working by wire drawing. The properties obtained with specimens of 0.081 inch diameter wire of typical alloy compositions consisting of 1.5% Ti, 2.5% Sn, 0.7% Cr, balance copper (Alloy A) and 1.5% Ti, 2.75% Sn, 0.7% Cr, balance copper (Alloy B) that were cold worked 64% and aged for varying periods up to 5 hours at 425° C. are summarized in Table I.

Table I

| Alloy | Aging time at 425° C. (hrs.) | Tensile strength (p.s.i.) | Yield strength (0.1% offset, p.s.i.) | Elongation (percent in 2 inches) | Electrical conductivity (percent I.A.C.S.) |
|-------|------------------------------|---------------------------|--------------------------------------|----------------------------------|--------------------------------------------|
| A     | 0                            | 108,000                   | 96,000                               | 2.5                              | 6.4                                        |
|       | 2                            | 121,500                   | 108,500                              | 8.0                              | 43.0                                       |
|       | 3                            | 120,000                   | 106,500                              | 9.0                              | 45.0                                       |
|       | 4                            | 119,000                   | 104,000                              | 10.0                             | 45.0                                       |
|       | 5                            | 116,000                   | 99,500                               | 9.0                              | 48.0                                       |
| B     | 0                            | 108,000                   | 96,000                               | 2.5                              | 6.5                                        |
|       | 2                            | 124,500                   | 110,000                              | 9.5                              | 41.0                                       |
|       | 3                            | 122,500                   | 107,500                              | 10.0                             | 42.0                                       |
|       | 4                            | 121,000                   | 107,000                              | 9.0                              | 43.0                                       |
|       | 5                            | 118,000                   | 102,500                              | 9.0                              | 43.5                                       |

From the foregoing, it becomes apparent that in the case of cold drawn wire subjected to appreciable cold working, the aging time for the development of optimum properties is actually between 2 to 3 hours at 425° C. Specimens cold drawn to reductions below about 40% were generally found to require close to 3 hours for obtaining electrical conductivities of at least 40% whereas those specimens that were cold drawn 53% or more attained over 40% I.A.C.S. electrical conductivity after aging for only approximately 2 hours.

Properties of 0.05 inch thick sheet were determined on a representative alloy containing 1.5% Ti, 2.5% Sn, 0.5% Cr, balance Cu, the material in this instance being processed by hot rolling, solution annealing and cold rolling to varying reductions from 16 to 80% after which the specimens were aged from 2 to 6 hours at 425 and 450° C. respectively. With cold rolling to reductions of 16.6, 28.6 and 37.5%, subsequent aging at either 425 or 450° C. generally resulted in electrical conductivities of at least 40% I.A.C.S. only after a heat treating time of 6 hours. With reductions of 50% or higher, however, conductivities of at least 40% I.A.C.S. were obtained after heat treating the cold rolled sheet material at 425° C. for generally from 4' to 6 hours. The heat treating time required at 450° C. is appreciably less as will be evident from the data submitted in Table II wherein other property values of the sheet material are listed.

Table II

## A. ALLOY COLD WORKED 50% (ROLLED)

| Aging temp. (°C.) | Heat treating time (hrs.) | Tensile strength (p.s.i.) | Yield strength (0.1% offset, p.s.i.) | Elongation (percent in 2 inches) | Hardness (VPN) | Electrical conductivity (percent I.A.C.S.) |
|-------------------|---------------------------|---------------------------|--------------------------------------|----------------------------------|----------------|--------------------------------------------|
| 425               | 0                         | 86,000                    | 80,000                               | 3.0                              | 203            | 8.0                                        |
| 425               | 2                         | 124,000                   | 108,000                              | 4.0                              | 282            | 28.0                                       |
| 425               | 3                         | 124,000                   | 107,000                              | 5.0                              | 282            | 28.0                                       |
| 425               | 4                         | 115,000                   | 95,000                               | 8.0                              | -----          | 39.0                                       |
| 425               | 5                         | 117,000                   | 100,000                              | 9.0                              | -----          | 40.0                                       |
| 425               | 6                         | 115,000                   | 95,000                               | 8.0                              | 250            | 40.0                                       |
| 450               | 3                         | 111,000                   | 92,000                               | 9.0                              | 250            | 40.0                                       |
| 450               | 6                         | 110,000                   | 88,000                               | 10.0                             | 239            | 43.0                                       |

## B. ALLOY COLD WORKED 66.5%

|     | 0 | 98,000  | 86,000  | 3.0  | 222   | 8.0  |
|-----|---|---------|---------|------|-------|------|
| 425 | 2 | 128,000 | 111,000 | 8.0  | ----- | 32.0 |
| 425 | 3 | 127,000 | 110,000 | 8.0  | 283   | 35.0 |
| 425 | 4 | 118,000 | 96,000  | 9.0  | ----- | 41.0 |
| 425 | 5 | 119,000 | 98,000  | 10.0 | ----- | 41.0 |
| 425 | 6 | 117,000 | 98,000  | 10.0 | ----- | 43.0 |
| 450 | 3 | 114,000 | 93,000  | 11.0 | 252   | 42.0 |
| 450 | 6 | 113,000 | 92,000  | 11.0 | 250   | 44.0 |

## C. ALLOY COLD WORKED 80%

|     | 0 | 107,000 | 90,000  | 3.0  | 235   | 8.0  |
|-----|---|---------|---------|------|-------|------|
| 425 | 2 | 127,000 | 109,000 | 8.0  | ----- | 37.0 |
| 425 | 3 | 126,000 | 109,000 | 8.0  | 287   | 39.0 |
| 425 | 4 | 119,000 | 100,000 | 11.0 | ----- | 42.0 |
| 425 | 5 | 119,000 | 98,000  | 11.0 | ----- | 43.0 |
| 425 | 6 | 116,000 | 95,000  | 10.0 | ----- | 43.0 |
| 450 | 3 | 114,000 | 94,000  | 12.0 | 253   | 43.0 |
| 450 | 6 | 114,000 | 93,000  | 11.0 | 250   | 44.0 |

A summary of the properties of a representative alloy of the present invention is presented in Table III wherein typical room temperature mechanical and physical properties of the alloy having the composition 1.5% Ti, 2.5% Sn, 0.5% Cr, balance Cu, are compared with those of beryllium copper having the composition 0.4% Be, 2.6% Co, balance Cu. It will be apparent that the room temperature properties of the respective alloys are quite comparable with respect to the materials (a) in solution annealed condition, (b) in the solution annealed and heat treated condition and also (c) in the solution annealed, cold worked and heat treated condition.

Table III

[Alloy Composition—1.5% Ti, 2.5% Sn, 0.5% Cr, balance Cu]

| 5  | Property                                                     | Sol. annealed at 875° C. quenched                              | Sol. annealed and heat treated at 450° C. for 6-8 hours    | Sol. annealed cold worked and heat treated at 450° C. for 6 hours <sup>1</sup> |
|----|--------------------------------------------------------------|----------------------------------------------------------------|------------------------------------------------------------|--------------------------------------------------------------------------------|
| 10 | Ult. tensile strength (p.s.i.)<br>0.2% offset<br>0.1% offset | 50-55,000<br>75-80,000<br>70-75,000<br>45-60,000<br>18,000,000 | 90-100,000<br>75-80,000<br>70-75,000<br>45-60,000<br>13-17 | 98-115,000<br>85-95,000<br>55-75,000<br>11                                     |
| 15 | Proportional limit (p.s.i.)                                  | 35-40                                                          | 37                                                         | 37                                                                             |
| 15 | Modulus of elasticity (p.s.i.)                               | -----                                                          | -----                                                      | -----                                                                          |
| 15 | Elongation (percent in 2 inches)                             | -----                                                          | -----                                                      | -----                                                                          |
| 15 | Ductility (percent reduction in area)                        | -----                                                          | -----                                                      | -----                                                                          |
| 15 | Vickers hardness (VPN)                                       | 80                                                             | 200-210                                                    | 230-250                                                                        |
| 15 | Electrical conductivity (percent I.A.C.S.)                   | 7                                                              | 40-48                                                      | 40-45                                                                          |
| 15 | Specific gravity (g./cm. <sup>3</sup> )                      | 8.8                                                            | -----                                                      | -----                                                                          |

20 1 0.05 inch thickness sheet material.

[Alloy Composition—0.4% Be, 2.6% Co, balance Cu]

| 25 | Property <sup>2</sup>                                        | Sol. annealed                      | Sol. annealed and heat treated       | Sol. annealed cold worked hard and heat treated |
|----|--------------------------------------------------------------|------------------------------------|--------------------------------------|-------------------------------------------------|
| 30 | Ult. tensile strength (p.s.i.)<br>0.2% offset<br>0.1% offset | 34-50,000<br>18-28,000<br>8-18,000 | 88-108,000<br>70-90,000<br>48-68,000 | 98-116,000<br>94-108,000<br>66-86,000           |
| 30 | Proportional limit (p.s.i.)                                  | 16-17,000,000                      | 8-15                                 | 5-12                                            |
| 30 | Modulus of elasticity (p.s.i.)                               | -----                              | 32                                   | -----                                           |
| 30 | Elongation (percent in 2 inches)                             | 20-35                              | 190-230                              | 210-240                                         |
| 35 | Ductility (percent reduction in area)                        | -----                              | 20-25                                | 45-48                                           |
| 35 | Vickers hardness (VPN)                                       | 65-85                              | -----                                | -----                                           |
| 35 | Electrical conductivity (percent I.A.C.S.)                   | 20-25                              | 48-52                                | 45-48                                           |
| 35 | Specific gravity (g./cm. <sup>3</sup> )                      | 8.8                                | -----                                | -----                                           |

2 2 Values from C.D.A. Publication No. 54 entitled "Beryllium Copper" issued in 1958 by the Copper Development Association.

40 The alloys of the present invention exhibit good ductility and strength at elevated temperatures as will be apparent from the properties listed in Table IV. The short time tensile properties of the 1.5% Ti, 2.5% Sn, 0.5% Cr, balance Cu, alloy in the form of 0.25 inch diameter rods were determined at 300 and 425° C. after 45 solution annealing at 875° C., quenching and heat treating at 450° C. for 6 hours.

Table IV

| 50 | Property                              | Testing temperature |            |
|----|---------------------------------------|---------------------|------------|
|    |                                       | 300° C.             | 425° C.    |
| 55 | Ultimate tensile strength (p.s.i.)    | 75,000              | 56,000     |
| 55 | Yield strength, 0.2% offset (p.s.i.)  | 66,000              | 51,000     |
| 55 | Yield strength, 0.1% offset (p.s.i.)  | 60,000              | 47,000     |
| 55 | Proportional limit (p.s.i.)           | -----               | 32,000     |
| 55 | Modulus of elasticity (p.s.i.)        | 20,500,000          | 21,000,000 |
| 55 | Elongation (percent in 2 inches)      | 11.0                | 16.0       |
| 55 | Ductility (percent reduction in area) | 60.0                | 31.0       |

60 By comparison, beryllium copper alloy having the composition 0.65% Be, 2.70% Co, balance copper, in the form of 0.25 inch diameter rod material processed by solution annealing at 920° C., quenching and heat treating at 480° C. for 3 hours and subsequently tested at the same temperatures possessed tensile strengths of 78,000 and 50,000 p.s.i. at 300 and 425° C. respectively. The modulus of elasticity of the beryllium copper alloy at 425° C. was 14,000,000 p.s.i. compared to the value of 21,000,000 p.s.i. shown in the above table for the quaternary alloy of the present invention. At 425° C., the proportional limit was only 18,000 p.s.i. for the beryllium-copper alloy compared to the value of 32,000 p.s.i. listed above. Contrasted with the elongation and ductility values for the new alloy listed in Table IV, the beryllium-copper alloy specimens tested at the same temperatures 75

were extremely brittle and the elongation and ductility values therefor were nil.

As previously indicated, silver may be additionally incorporated in the quaternary alloy in amounts up to about 1% without materially effecting the properties of the resulting alloy. The properties obtained with 0.132 inch diameter wire treated as set forth below and made with alloys of the composition 1.5% Ti, 2.5% Sn, 0.6% Cr with amounts of silver ranging from 0.2 to 1%, the balance being copper are summarized in Table V.

Table V

| Percent, Ag | Treatment                    | Ultimate tensile strength (p.s.i.) | Yield strength (0.1% offset, p.s.i.) | Elong. (percent in 2 inches) | Elec. cond. (percent I.A.C.S.) |
|-------------|------------------------------|------------------------------------|--------------------------------------|------------------------------|--------------------------------|
| 0.2         | Sol. ann. at 875° C. 30 min. | 58,000                             | 22,000                               | 36.4                         | 7.2                            |
|             | Aged at 450° C. for 2 hours  | 99,500                             | 79,000                               | 11.5                         | 17.8                           |
|             | Aged at 450° C. for 6 hours  | 95,000                             | 72,000                               | 11.0                         | 37.6                           |
|             | Aged at 450° C. for 8 hours  | 93,000                             | 67,000                               | 15.0                         | 42.5                           |
|             | Aged at 450° C. for 14 hours | 88,000                             | 63,000                               | 16.0                         | 47.3                           |
|             | Sol. ann. at 875° C. 30 min. | 58,000                             | 23,000                               | 33.0                         | 7.0                            |
| 0.5         | Aged at 450° C. for 2 hours  | 85,000                             | 63,000                               | 13.0                         | 19.0                           |
|             | Aged at 450° C. for 6 hours  | 86,000                             | 65,000                               | 14.5                         | 37.6                           |
|             | Aged at 450° C. for 8 hours  | 87,000                             | 64,000                               | 14.0                         | 38.3                           |
|             | Aged at 450° C. for 14 hours | 86,000                             | 62,000                               | 18.0                         | 46.5                           |
|             | Sol. ann. at 875° C. 30 min. | 57,000                             | 22,000                               | 36.0                         | 6.7                            |
|             | Aged at 450° C. for 2 hours  | 100,000                            | 80,000                               | 9.0                          | 18.2                           |
| 0.8         | Aged at 450° C. for 6 hours  | 94,000                             | 70,000                               | 11.5                         | 36.6                           |
|             | Aged at 450° C. for 8 hours  | 92,000                             | 66,000                               | 14.0                         | 41.0                           |
|             | Aged at 450° C. for 14 hours | 88,000                             | 64,000                               | 11.5                         | 48.2                           |
|             | Sol. ann. at 875° C. 30 min. | 58,000                             | 22,000                               | 38.0                         | 7.3                            |
|             | Aged at 450° C. for 2 hours  | 98,000                             | 78,000                               | 6.0                          | 19.0                           |
|             | Aged at 450° C. for 6 hours  | 93,000                             | 68,000                               | 14.0                         | 41.6                           |
| 1.0         | Aged at 450° C. for 8 hours  | 93,000                             | 66,000                               | 14.0                         | 42.0                           |
|             | Aged at 450° C. for 14 hours | 87,000                             | 62,000                               | -----                        | 47.3                           |

Small amounts of phosphorus added to the alloy made with initially oxygen-free copper depress the electrical conductivity appreciably indicating that the phosphorus stays in alpha solid solution. From 0.02 to 0.05% phosphorus added to the alloy made with initially oxygen-free copper lowers the conductivity of the alloy containing 1.5% Ti, 2.5% Sn, 0.5% Cr, from 45 to 35-37% I.A.C.S. but the strength of the alloy is not affected to any appreciable extent.

The foregoing alloys were all made with initially oxygen-free copper. It was found that the tensile properties of the alloy made using tough pitch copper are generally about the same as those of the corresponding alloy made with initially oxygen-free copper provided that both alloys are processed in the same manner. The electrical conductivity is somewhat lower, however, as illustrated by the alloys containing 1.5% Ti, 2.5% Sn, 0.5% Cr. Comparison of the properties of the similarly processed alloys made with initially oxygen-free and tough pitch coppers showed a depression in electrical conductivity of from 45 to 37% I.A.C.S. attributable to the presence of Cu<sub>2</sub>O in the tough pitch copper. Accordingly, the use of initially oxygen-free copper is generally necessary for obtaining electrical conductivities above 40% I.A.C.S.

While the present invention has been described herein in considerable detail with reference to specific embodiments thereof, it is not desired to be limited thereby but it is intended to cover the invention broadly within the scope of the appended claims.

What is claimed is:

- An age hardenable copper base alloy of at least 90% copper content, said alloy consisting essentially of from 0.3 to 4% titanium, 0.5 to 5% tin and 0.05 to 2% chromium, the balance being substantially all copper with incidental impurities normally associated therewith.
- An age hardenable copper base alloy of at least 90% copper content, said alloy consisting essentially of from 1 to 3% titanium, 2 to 4% tin and 0.2 to 0.8% chromium, the balance being copper with incidental impurities normally associated therewith.
- An age hardenable copper base alloy of at least 95% copper content, said alloy consisting essentially of from 1.3 to 1.7% titanium, 2.2 to 2.9% tin and 0.3 to 0.6% chromium, the balance being copper with incidental impurities normally associated therewith.
- An age hardenable copper base alloy of at least 95% copper content, said alloy consisting essentially of from 1.3 to 1.7% titanium, 2.2 to 2.9% tin and 0.3 to 0.6% chromium, the balance being initially oxygen-free copper, the titanium and tin being present in the alloy in the ratio of about 1:1.7 respectively.
- An age hardenable copper base alloy of at least 90% copper content, said alloy consisting essentially of from 1 to 3% titanium, 2 to 4% tin, 0.2 to 0.8% chromium and an additional alloying element selected from the group consisting of silver and phosphorus in the amounts not exceeding 1% and 0.05% respectively, the balance of the alloy being substantially all copper with incidental impurities normally associated therewith.
- An age hardenable copper base alloy consisting essentially of from 1 to 3% titanium, 2 to 4% tin, 0.2 to 0.8% chromium and the balance substantially initially oxygen-free copper with impurities normally associated with such copper.
- An age hardened alloy consisting essentially of from about 1.3 to 1.7% titanium, about 2.2 to 2.9% tin, about 0.3 to 0.6% chromium, the balance being substantially all initially oxygen-free copper with impurities normally associated with such copper, said alloy being characterized by a combination of properties including a tensile strength of at least 90,000 p.s.i. and electrical conductivity of at least 40% I.A.C.S.
- Copper-titanium-tin-chromium alloy made with initially oxygen-free copper, the content of titanium, tin and chromium of the quaternary alloy being about 1.5, 2.5 and 0.5% respectively, said alloy in the cold worked and aged condition being characterized by a minimum tensile strength of 110,000 p.s.i. and electrical conductivity above 40% I.A.C.S.

#### References Cited in the file of this patent

#### UNITED STATES PATENTS

- 2,059,557 Corson ----- Nov. 3, 1936  
 2,189,198 Comstock ----- Feb. 6, 1940  
 2,797,300 Hawthorne ----- June 25, 1957

#### FOREIGN PATENTS

- 812,407 Great Britain ----- Apr. 22, 1959